

1

2,854,327

**EXOTHERMIC CHROMIUM COMPOUND CONTAINING COMPOSITION AND METHOD OF MAKING SAME**

Tom S. Perrin and Howard E. Everson, Painesville, and Harry B. Kinnear, Columbus, Ohio, assignors, by direct and mesne assignments, to Diamond Alkali Company, Cleveland, Ohio, a corporation of Delaware

No Drawing. Application February 12, 1954  
Serial No. 410,042

26 Claims. (Cl. 75—27)

This invention relates to a method for recovering chromium metal, and more particularly relates to a method for recovering chromium metal alone or in combination with other metals, such as a chromium-bearing alloy, and still more particularly relates to the recovery of chromium metal from a mixture of an alkaline earth metal chromate with complex chromium compounds obtained by the reaction of an alkali metal chromate with reducing agents which reduce the chromium to valences apparently intermediate its normal 3 and 6 valent states, and relates as well to exothermically reacting compositions containing an alkaline earth metal chromate and the said complex chromium compounds.

In the manufacture of chromium alloy steels, the chromium of the steel may be obtained by dissolving an alloy, such as ferrochromium, in the molten steel bath. The procedure of dissolving the alloy in the bath, however, has distinct disadvantages to the steel maker, in that the time required to dissolve an alloy, such as ferrochromium, in the bath is excessive, during which time there is danger that the bath composition will change. For example, the bath may become contaminated by nitrogen absorbed from the furnace atmosphere, and if an electric arc furnace is used, there is additional likelihood of carbon being absorbed into the bath.

The art, therefore, has sought other means for introducing chromium into alloy baths. One such means is a composition containing a chromium alloy, an oxidizing agent, and a reducing agent comprising slag-forming components. By properly combining the components of such a composition, the exothermic reaction of oxidizing and reducing agents may generate sufficient heat to provide molten chromium or an alloy thereof in contact with the steel bath, whereby rapid solution of chromium, or the alloy, in the bath takes place.

Compositions of matter which undergo an exothermic chemical reaction to produce metallic elements and alloys, referred to in the art as "exothermic mixes," have in general included as the oxidizing agent, sodium nitrate or sodium chloride, together with a reducing agent, such as silicon, calcium, aluminum, and magnesium, either alone or in the form of an alloy with ferrous or non-ferrous metals. Such exothermic mixes have been used in the manufacture of steel for the purpose of introducing chromium and other metallic elements into a molten steel bath, either in the furnace or in the ladle.

The difficulties encountered in the manufacture of steel with the prior art exothermic mixes containing sodium nitrate includes the introduction of nitrogen into the molten steel bath, which nitrogen, if excessive, in some types of chromium-bearing steels, causes the ingots poured from the bath to rise in the mold and "bleed," even where such exothermic mixes may be used in the production of relatively low chromium-containing steel.

Usually, in the use of oxidizing agents such as sodium nitrate, sodium or potassium chloride, and the like, the chromium in the exothermic mixes is associated with

2

one or more components of the reducing agent in the form of an alloy, such as commercial grades of ferro-chrome silicon (Cr 35—40%, Si 42%—50%) wherein silicon is the slag-forming component and the reducing agent. Other metals, such as Ca and Al, may also be included in the form of their alloys, such as calcium silicide, or ferrochrome-silicon-aluminum, and the like, as slag-forming and reducing agent components.

The problem faced in the art has been one of providing exothermic mixes containing low cost sources of chromium and oxidizing agents which do not produce deleterious gases in the steel bath, while providing a reaction sufficiently exothermic that chilling of the steel bath is not encountered.

The present invention is based in part upon the finding that complex chromium compounds may be produced by the reaction of an alkali metal chromate with substances such as hydrogen, carbon, carbon monoxide, or compounds having hydrogen chemically combined with carbon, in a non-oxidizing atmosphere, which compounds are apparently in a state of oxidation intermediate that that of the trivalent and hexavalent forms of chromium. Further, the present invention is based upon the finding that such reaction products will, under proper conditions, react exothermically with certain metal or metalloid reducing agents to produce metallic chromium, and that such reaction is sufficiently exothermic to be useful either in the recovery of chromium metal as such, or in combination with other alloying elements, such as in the manufacture of chromium-bearing steel. Moreover, since such reaction products are substantially free from sulfur compounds, and may be produced substantially free from carbon, alloys low in sulfur and carbon are readily produced in accordance with this invention.

Further, the present invention is based upon the finding that the rate of reaction of such complex chromium compounds with certain metal or metalloid reducing agents is accelerated and readily controlled by the addition, to a mixture of such materials, of an alkaline earth metal chromate, for example, calcium chromate, and that such reaction products will, under proper conditions react exothermically with certain metal or metalloid reducing agents to produce metallic chromium, and that such reaction is sufficiently exothermic and efficient to give unusually high yields of chromium metal, either in the recovery of chromium metal as such, or in combination with other alloying elements, such as in the manufacture of chromium-bearing steel.

The said complex chromium compounds, upon which the present invention is based in part, appear to be a chemical combination of two or more chromium-containing components which are already saturated according to the classical concepts of valency. Such complexes are believed to contain chromium in a valence state intermediate the normal trivalent and hexavalent states of this element, since they may be characterized by (1) their ability to yield both trivalent and hexavalent chromium compounds on being calcined at temperatures of the order of about 980°—1000° C., in an oxidizing atmosphere, (2) their relative chemical inertness except under strong oxidizing conditions, (3) insolubility in water, and (4) other properties which are not characteristic of physical mixtures of trivalent and hexavalent chromium compounds. The present application is related to application Ser. No. 410,041, filed February 12, 1954, in the name of Tom S. Perrin and Howard E. Everson.

One of the objects of the present invention is to provide exothermic mixes containing an alkaline earth metal chromate in admixture with complex chromium compounds wherein the chromium is apparently in an intermediate state of oxidation between that of trivalent and

hexavalent chromium, whereby the oxidizing agent of the exothermic mix is used as a source of chromium and contamination by deleterious gases of the metal produced is prevented.

A further object of the invention is to provide exothermic mixes containing the said complex chromium compounds mixed with an alkaline earth metal chromate, as the oxidizing agent of such mixes, whereby unusually efficient and economic recovery of chromium metal from such mixes is obtained.

Another object of the invention is to provide an exothermic mix from which chromium metal may be recovered alone or in combination with other metals in an alloy solution.

These and other objects of the invention will be apparent from the description of the invention given hereinbelow.

Pursuant to the above objects, the present invention includes exothermic alloying compositions comprising, as the oxidizing agent thereof, a mixture of alkaline earth metal chromate with a complex chromium compound obtained by the reaction of an alkali metal chromate, in the form of a solid, as opposed to a solution, with a substance selected from the group consisting of hydrogen, carbon, carbon monoxide, and compounds having hydrogen chemically combined with carbon, in a non-oxidizing atmosphere, and comprising as the reducing agent thereof at least one element from the group consisting of alkaline earth metals, Al, and Si. The invention also includes the method of recovering chromium which comprises mixing an alkaline earth metal chromate and a complex chromium compound obtained by the reaction of an alkali metal chromate, in the form of a solid, as opposed to a solution, with a substance selected from the group consisting of hydrogen, carbon, carbon monoxide, and compounds having hydrogen chemically combined with carbon, in a non-oxidizing atmosphere, with at least one element selected from the group consisting of alkaline earth metals, Al, and Si, heating the mixture to effect reaction between said alkaline earth metal chromate, said reaction product, and an element of said group, and recovering chromium from the reaction products of said mixture. The term "alkaline earth metals" refers to the group II elements, Mg, Ca, Sr, Ba, and Ra, and the term "alkaline earth metal chromates" refers to the chromate salts of these metals. The order of preference, both for alkaline earth metals and their chromate salts, in the present invention is Ca, Mg, Sr, Ba, and Ra.

The complex chromium compounds which are products obtained by the solid-phase reaction of an alkali metal chromate with a substance selected from the group consisting of hydrogen, carbon, carbon monoxide, and compounds having hydrogen chemically combined with carbon, in a non-oxidizing atmosphere, may be obtained from any one of the alkali metal chromates, such as lithium, sodium, potassium, rubidium, and cesium chromate. Preferably, however, for the purposes of the present invention, such reaction products are obtained by the solid-phase reaction of sodium chromate with hydrogen or a compound having hydrogen chemically combined with carbon. These reaction products are preferably obtained at temperatures above 250° C. and below the fusion point of the reaction mass.

Hydrogen, which may be employed in the preparation of the preferred complex reaction products, may be derived from any suitable source of hydrogen, such as from the electrolysis of sodium chloride brine or other aqueous solution of an electrolyte. Similarly, the carbon, carbon monoxide, or compounds containing hydrogen chemically combined with carbon may be any suitable material readily entering into reaction with the solid alkali metal chromate, such as, for example, charcoal, graphite, coke, producer gas, coke oven gas, carbohydrates, of which sawdust, wood flour, sugars, starch, and the like are representative, and hydrocarbons, preferably in the gaseous

state, of which the lower aliphatic hydrocarbons, both saturated and unsaturated, are representative, may be employed. The solid-phase reaction product of an alkali metal chromate with carbon, or one of the above carbon compounds, may suitably be used where the introduction of carbon into the steel bath is not deleterious.

The metalloid and metal reducing agents as noted hereinabove, include the alkaline earth metals, Mg, Ca, Sr, Ba, and Ra, as well as Al and Si. These reducing agents, hereinafter referred to as reductants, may, if desired, be employed alone, but preferably are employed in combination with other metallic elements as alloys, and especially suitable are those alloys in which silicon is present. Thus, alloys such as the various commercial forms of ferrosilicon, ferrochrome silicon, ferrochrome silicon aluminum, ferrosilicon aluminum (Alsifer), aluminum silicide, calcium silicide, calcium aluminum silicide, and the like, may be used.

In accordance with the present invention, the complex chromium compounds referred to above together with an alkaline earth metal chromate, preferably calcium chromate, comprise the oxidizing agent of the exothermic mixes. The proportion of the chromium available from the alkaline earth metal chromate to the chromium available from the complex chromium compounds, in the oxidizing portion of the exothermic mixes, may be varied as desired, but preferably is above about 1:10 and up to 1:3, i. e., the amount of chromium available from the alkaline earth metal chromate is preferably substantially above about  $\frac{1}{10}$  and up to about  $\frac{1}{3}$  that available from the complex chromium compounds.

Where the proportion of chromium from the alkaline earth metal chromate to the chromium from the complex chromium compounds is substantially less than 1:10, the combined effect of the accelerated reaction and the control thereof in a manner to bring about maximum yields of chromium metal either as such or as an alloy, is not realized. Also where the proportion of chromium from the alkaline earth metal chromate to the chromium from the complex chromium compounds is substantially greater than 1:3, the exothermic reaction may become sufficiently violent that an appreciable loss of material from the reaction mass is encountered, and appreciably lower recovery of chromium from the exothermic mix may result, especially where calcium chromate is the alkaline earth metal chromate employed and aluminum is used as one of the components of the reductant portion of the exothermic mix.

In order to determine the amount of reductant which may suitably be employed in the compositions and in the practice of the method of the present invention, the oxidizing power of the complex chromium compounds which may conveniently be considered as available for reaction with the above-noted reducing agents, is computed by arbitrarily converting the Cr content of the complex chromium compounds to  $\text{Cr}_2\text{O}_3$ , and proportioning the calculated amount of oxygen available therefrom to the amounts of the reductants with which it may be combined.

Thus, for example, if a chromium complex material were prepared as described hereinabove, and were found to contain 54.7% Cr (total), this would be the equivalent of 80%  $\text{Cr}_2\text{O}_3$ , which would be taken (arbitrarily) to represent the portion of the chromium complex material available for oxidizing the reducing agents. If then the significant components of the reductant were Al and Si, for example, it might be desirable to proportion the Al component to the equivalent of all of the alkaline earth metal chromate and  $\frac{1}{3}$  the  $\text{Cr}_2\text{O}_3$ , and the Si to the equivalent of  $\frac{2}{3}$  the  $\text{Cr}_2\text{O}_3$ . Since the reactions involved for the  $\text{Cr}_2\text{O}_3$  may be represented thus:



and



the computations are conveniently set up thus:

$$\frac{(2)(27) \text{ (Amt. Cr}_2\text{O}_3)}{(152)} \times \frac{1}{3} = x \text{ (Al)}$$

$$\frac{(3)(28) \text{ (Amt. Cr}_2\text{O}_3)}{(2)(152)} \times \frac{2}{3} = y \text{ (Si)}$$

The amounts of the components of the reductant indicated by such computation ( $x$  and  $y$ ) are preferably increased by a factor within the range of 1.1 to 2.5, suitably by a factor of 1.5 to 1.75.

It will, of course, be apparent to those skilled in the art that the alkaline earth metal chromate may be considered to react with the reducing agent in the normal manner, to produce chromium metal, calcium oxide, and the oxide of the reducing agent. The amount of reducing agent, Al in the example above, equivalent to the alkaline earth metal chromate is computed in accordance with well-known principles for calculating equivalents in oxidation-reduction equations. The amounts of the components of the reductant indicated by the computation for the specific alkaline earth metal chromate employed, are also preferably increased by a factor substantially within the range of 1.1 to 2.5, and suitably by a factor of 1.5 to 1.75.

One reason for employing an excess of the reductant over the calculated amount for the complex chromium compounds arises, in part, from the fact that the oxygen combined with chromium in the complex chromium compounds is in excess of that required to satisfy the formula  $\text{Cr}_2\text{O}_3$ , and the chromium, therefore, as noted above, would appear to be in a valence state intermediate that of the normal trivalent or hexavalent state, or possibly to be combined with oxygen and alkali metal in some coordinate co-valent state. Another reason arises when silicon is used as one of the components of the reductant. There is evidence reported in the chemical literature indicating that reaction of oxygen-bearing compounds and silicon at high temperatures may result in silicon-oxygen compounds having less than two atoms of oxygen per atom of silicon.

The higher recovery of chromium where the excess of reductants, as computed above, is of the order of 1.5 to 1.75, would tend to indicate that the first of these reasons is sound, and where silicon is one component of the reductants, that the second reason may also be sound.

In the preparation of the compositions of the present invention, as well as in the method thereof, the complex chromium compounds, and the reductants, are preferably in a finely divided state, and are mixed together so as to form uniform dispersion of both components. The mixture may be combined with a suitable binding agent and subjected to mechanical agglomeration, as by briquetting or pelletizing, or may be used in the form of loose, free-flowing powder.

Where the compositions of the present invention are employed as a means of making final adjustments in the chromium content of steel in the ladle, such compositions are preferably in the form of a loose, free-flowing powder. Where larger amounts of chromium are desired in ladle additions, the compositions of the present invention may be used in the form of briquettes, for example, by placing the briquettes in the ladle prior to tapping the steel into the ladle.

In order that those skilled in the art may better understand the nature of the compositions and the method of the present invention and in what manner the same may be carried into effect, the following specific examples are offered:

#### Example I

100 parts of ingot iron are placed in the crucible of a high frequency induction furnace, and melted. Furnace additions of 0.25% silicon and 0.35% manganese, as

ferrosilicon and ferromanganese, respectively, are made when the melt reaches the temperature of about 1590° C. Within about 1/2 minute after the addition of the ferrosilicon and ferromanganese, a sample is poured for chemical analysis. After pouring the base metal sample, the temperature of the metal in the furnace is allowed to rise again to about 1590° C., and the power adjusted to maintain this temperature.

2.2 parts of the reaction product of sodium chromate and gaseous hydrogen, which reaction product, upon analysis, and computing the chromium and sodium content thereof in terms of  $\text{Cr}_2\text{O}_3$  and  $\text{Na}_2\text{O}$  as described hereinabove, gives:  $\text{Cr}_2\text{O}_3$ , 77.7% and  $\text{Na}_2\text{O}$ , 13.2%, are dry-mixed with calcium chromate 0.93 part, atomized aluminum 0.70 part, and ferrochrome silicon 1.32 parts, giving 5.15 parts of an exothermic mix containing 38.8% chromium. The aluminum is proportioned so as to be equivalent to 1.5 times the calcium chromate, plus about 0.5 of the computed  $\text{Cr}_2\text{O}_3$  content of the chromium complex. The silicon is proportioned so as to be equivalent to about 1.2 times the computed  $\text{Cr}_2\text{O}_3$  content of the chromium complex.

The temperature of the metal bath in the furnace is increased to about 1760° C., and about 1/2 of the bath is tapped into a preheated ladle. The 5.15 parts of the exothermic mixture described above are then introduced into the ladle in the form of a loose powder, whereupon the exothermic reaction is initiated and is found to be complete within about 1/2 minute. The remainder of the metal bath is then tapped into the ladle. The slag produced by the exothermic mix is fluid, and analysis of the bath in the ladle shows that the silicon content thereof, after the addition of the exothermic mixture is 0.34%, and that the chromium content thereof is 1.72%, showing an 87.5% recovery of the chromium in the exothermic mixture. The total amount of all metal recovered from the furnace and ladle is 103 parts.

#### Example II

Following essentially the same procedure as that described for Example I above, for the addition of silicon and manganese, a heat is prepared consisting of 100 parts of ingot iron, which is charged to a high frequency induction furnace. 2.77 parts of the reaction product of sodium chromate and hydrogen, which reaction product, upon analysis, and computing the chromium and sodium contents thereof in terms of  $\text{Cr}_2\text{O}_3$  and  $\text{Na}_2\text{O}$  as in Example I above, gives: 70.7%  $\text{Cr}_2\text{O}_3$  and 23.4%  $\text{Na}_2\text{O}$ , are dry mixed with 0.82 part of calcium chromate, 0.39 part of atomized aluminum, and 2.3 parts of ferrochrome silicon, containing 41% Si, giving 6.27 parts of an exothermic mix containing 40.5% Cr. The aluminum is proportioned so as to be equivalent to 1.5 times the calcium chromate of the exothermic mix, and the silicon of the ferrochrome silicon is proportioned to be equivalent to 1.75 times the computed  $\text{Cr}_2\text{O}_3$  content of the chromium complex.

After the temperature of the molten metal bath in the furnace has reached about 1590° C., the furnace is tapped for a sample for analysis, which analysis shows that the bath contains 0.22% of Si, and 0.01% of Cr. The bath in the furnace is heated to a temperature of about 1760° C., and about half of the bath is tapped into a preheated ladle. The 6.3 parts of the exothermic mixture described above are then introduced into the ladle in the form of a loose powder, whereupon the exothermic reaction is initiated and is found to be complete within about 1 1/2 minutes. The slag formed by the exothermic mix is fairly viscous, at this point, and the remainder of the metal in the furnace is then tapped into the ladle. The metal is separated from the slag, and analysis of the bath in the ladle shows that the silicon content thereof has increased to 0.79%, and the chromium content thereof has increased to 2.53%, giving a 93.2% recovery of the chromium in the exothermic mix.

*Example III*

Following essentially the same procedure as that described for Example II above, for the addition of silicon and manganese, a heat is prepared consisting of 200 parts of ingot iron which is charged to a high frequency induction furnace, and sufficient ferrosilicon and ferromanganese added thereto to provide the same amounts of silicon and manganese as that prescribed in Example II. 11.3 parts of the same chromium complex material as that used in Example II are dry-mixed with 3.15 parts of calcium chromate, 1.5 parts of atomized aluminum, and 8.81 parts of ferrochrome silicon containing 41% Si, giving 24.76 parts of an exothermic mixture containing 40.5% Cr. The aluminum in the exothermic mixture is proportioned so as to be equivalent to 1.5 times the calcium chromate content thereof, and the silicon in the ferrochrome silicon of the exothermic mix is proportioned to be equivalent to about 1.65 times the computed  $\text{Cr}_2\text{O}_3$  content of the chromium complex.

After the temperature of the molten metal bath in the furnace has reached 1590° C., the furnace is tapped for a sample for analysis, which analysis shows that the bath contains 0.22% Si and 0.02% Cr. The bath in the furnace is then heated to a temperature of about 1760° C., and about 1/2 of the bath is tapped into a preheated ladle. The 24.76 parts of the exothermic mix are then added to the ladle in the form of a loose powder, whereupon reaction is initiated and found to be complete within about 1.5 minutes. The remainder of the metal bath is then tapped into the ladle. The slag produced by the exothermic mix is fairly fluid, and analysis of the bath in the ladle shows that the silicon content thereof after the addition of the exothermic mixture is 0.8%, and the chromium content thereof is 4.36%, giving a 94.2% recovery of chromium in the exothermic mix.

*Example IV*

Following the procedure of Example II above, 200 parts of ingot iron, and sufficient ferrosilicon and ferromanganese to give a 0.25% silicon and 0.35% manganese before the addition of the exothermic mix, are heated in a high frequency induction furnace.

22.6 parts of the reaction product of hydrogen and sodium chromate, prepared as in Example I above, which reaction product, upon analysis, and computing the Cr and Na in terms of  $\text{Cr}_2\text{O}_3$  and  $\text{Na}_2\text{O}$ , as in Example II, gives  $\text{Cr}_2\text{O}_3$  70.7% and  $\text{Na}_2\text{O}$  23.6%, are dry-mixed with 6.3 parts of calcium chromate, 3.0 parts of atomized aluminum, and 17.6 parts of ferrochrome silicon to make an exothermic mixture containing 40.5% Cr.

About 1/2 of the molten metal bath, at about 1760° C. is tapped into a preheated ladle. The exothermic mixture in loose form is then placed on top of the metal. Reaction is initiated substantially immediately and the reaction completed within about 2 minutes, yielding a fluid slag. The remainder of the bath in the furnace is tapped into the ladle. The amount of aluminum added in the exothermic mixture is proportioned to be equivalent to 1.5 times the calcium chromate present. The amount of silicon added as ferrochrome silicon in the exothermic mix is proportioned to be equivalent to about 1.5 times the computed  $\text{Cr}_2\text{O}_3$  of the chromium complex. A sample of the final bath is tapped from the ladle and analyzed. The analysis shows 0.08% carbon, 1.81% silicon, and 9.40% chromium, representing a 96.1% recovery of chromium from the exothermic mixture.

*Example V*

Following the procedure of Example II above, 100 parts of ingot iron, and sufficient ferrosilicon and ferromanganese, to give a 0.25% silicon and 0.35% manganese before the addition of the exothermic mix, are heated in a hot high frequency induction furnace.

2.77 parts of the exothermic mix employed in Ex-

amples II, III, and IV above, are dry-mixed with 0.82 part of calcium chromate, 0.38 part of atomized aluminum, and 2.29 parts of ferrochrome silicon containing 41% Si, giving an exothermic mixture containing 40.5% Cr.

A sample is tapped from the molten metal in the furnace, and analyzed, and found to contain 0.3% Si, and 0.03% Cr. The temperature of the molten metal bath in the furnace at the time of sampling is about 1590° C., the metal bath is heated to a temperature of about 1760° C., and about 1/2 of the bath is tapped into a preheated ladle. The exothermic mixture (6.26 parts) in the form of a loose powder is then placed on top of the molten metal. Reaction is initiated substantially immediately and the reaction is complete within about 1 1/4 minutes. The remainder of the bath in the furnace is tapped into the ladle, and the slag is noted to be somewhat viscous.

The amount of aluminum in the exothermic mixture is proportioned to be equivalent to about 1.5 times the amount of calcium chromate in the exothermic mix, and the silicon in the ferrochrome silicon is proportioned to be equivalent to about 1.75 times the computed  $\text{Cr}_2\text{O}_3$  content of the complex chromium compound.

The metal bath is separated from the slag and a sample of the final bath is tapped from the ladle for analysis. The analysis shows that the silicon content of the metal has increased to 0.69%, and that the chromium content has increased to 2.43%, giving a 98.5% recovery of chromium in the complex chromium compound.

In each of Examples I through V, the temperature of the metal bath rises consistently a minimum of 50°-60° C., from the time of addition of the exothermic mix to the ladle up to the time when the exothermic reaction is apparently completed.

While there have been described various embodiments of the invention, the methods and products described are not intended to be understood as limiting the scope of the invention as it is realized that changes therewithin are possible and it is further intended that each element recited in any of the following claims is to be understood as referring to all equivalent elements for accomplishing substantially the same results in substantially the same or equivalent manner, it being intended to cover the invention broadly in whatever form its principle may be utilized.

What is claimed is:

1. An exothermic composition comprising as the oxidizing agent thereof, an alkaline earth metal chromate, and the reaction product obtained by the solid-phase reaction, in a nonoxidizing atmosphere, of an alkali metal chromate with a substance selected from the group consisting of hydrogen, carbon, carbon monoxide, and compounds having hydrogen chemically combined with carbon, said solid-phase reaction taking place at a temperature above 250° C., and below the fusion point of the reaction mass, the chromium of said reaction product being in an intermediate state of oxidation between that of trivalent and hexavalent chromium, and comprising as the reducing agent thereof an element selected from the group consisting of the alkaline earth metals, aluminum and silicon.

2. The composition of claim 1 in which said reaction product is the product obtained by the solid-phase reaction of an alkali metal chromate with hydrogen.

3. The composition of claim 1 in which said reaction product is the product obtained by the solid-phase reaction of an alkali metal chromate with carbon.

4. The composition of claim 1 in which said reaction product is the product obtained by the solid-phase reaction of an alkali metal chromate with carbon monoxide.

5. The composition of claim 1 in which the said reaction product is the product obtained by the solid-phase reaction of an alkali metal chromate with a compound having hydrogen chemically combined with carbon.

6. The composition of claim 1 in which said alkali metal chromate is sodium chromate.

7. The composition of claim 6 in which said reaction product is the product obtained by the solid-phase reaction of sodium chromate with hydrogen.

8. The composition of claim 6 in which said reaction product is obtained by the solid-phase reaction of sodium chromate with carbon.

9. The composition of claim 6 in which said reaction product is the product obtained by the solid-phase reaction of sodium chromate with carbon monoxide.

10. The composition of claim 6 in which said reaction product is obtained by the solid-phase reaction of sodium chromate and a compound having hydrogen chemically combined with carbon.

11. The composition of claim 6 in which said alkaline earth metal chromate is calcium chromate.

12. The method of recovering chromium which includes the steps of mixing an alkaline earth metal chromate, and the reaction product obtained by the solid-phase reaction, in a non-oxidizing atmosphere, of an alkali metal chromate and a substance selected from the group consisting of hydrogen, carbon, carbon monoxide, and a compound having hydrogen chemically combined with carbon, said solid-phase reaction taking place at a temperature above 250° C., and below the fusion point of the reaction mass, the chromium of said reaction product being in an intermediate state of oxidation between that of trivalent and hexavalent chromium, with at least one element selected from the group consisting of alkaline earth metals, aluminum, and silicon, and heating the mixture to effect reaction between said alkaline earth metal chromate, said reaction product, and said element of said group.

13. The method of claim 12 in which said reaction product is obtained by the solid-phase reaction of an alkali metal chromate with hydrogen.

14. The method of claim 12 in which said reaction product is obtained by the solid-phase reaction of alkali metal chromate with carbon.

15. The method of claim 12 in which said reaction product is obtained by the solid-phase reaction of an alkali metal chromate with carbon monoxide.

16. The method of claim 12 in which said reaction product is obtained by the solid-phase reaction.

17. The method of claim 12 in which said reaction product is obtained by the solid-phase reaction of alkali metal chromate with a compound having hydrogen chemically combined with carbon.

18. The method of claim 12 in which said alkali metal

chromate is sodium chromate, and said alkaline earth metal chromate is calcium chromate.

19. The method of claim 18 in which the material selected from the group consisting of alkaline earth metals, aluminum and silicon, is equivalent to 1.1 to 2.5 times the sum of the calcium chromate, and the Cr content of said product calculated as  $\text{Cr}_2\text{O}_3$ .

20. The method of manufacturing a chromium-bearing alloy which includes the steps of reacting, in a non-oxidizing atmosphere, solid sodium chromate with a substance selected from the group consisting of hydrogen, carbon, carbon monoxide, and compounds having hydrogen chemically combined with carbon, at a temperature above about 250° C., and below the fusion point of the reaction

15 mass, the chromium of the reaction product thus obtained being in an intermediate state of oxidation between that of trivalent and hexavalent chromium, mixing said reaction product with an alkaline earth metal chromate, and a non-carbonaceous reducing agent selected from the

20 group consisting of the alkaline earth metals, aluminum and silicon, to form an exothermically reacting mixture, the amount of said reducing agents being within the range of 1.1 to 2.5 times that amount equivalent to the alkaline earth metal chromate and the available oxygen of said

25 reaction product, said available oxygen being computed as  $\text{Cr}_2\text{O}_3$  from the total Cr content of said reaction product, combining said exothermically reacting mixture with a molten metal bath with which the chromium is to be alloyed, allowing the reaction between said reaction product and said reducing agents to proceed substantially to completion, and recovering a chromium-bearing alloy from said molten bath.

21. The method of claim 20 in which said alkaline earth metal chromate is calcium chromate.

35 22. The method of claim 21 in which said reducing agents include silicon.

23. The method of claim 21 in which said reducing agents include an alloy of silicon.

40 24. The method of claim 23 in which said alloy of silicon is ferrochrome silicon.

25. The method of claim 23 in which said reducing agents include calcium.

26. The method of claim 25 in which said alloy of silicon is calcium silicide.

45

References Cited in the file of this patent

UNITED STATES PATENTS

2,332,415 Udy \_\_\_\_\_ Oct. 19, 1943  
2,587,552 Vedensky \_\_\_\_\_ Feb. 26, 1952